

Patented Nov. 8, 1927.

## UNITED STATES PATENT OFFICE.

JOHN H. MITCHELL, OF HABANA, CUBA.

## COMPOSITION PAPER OR PULP BOARD AND METHOD OF MAKING THE SAME.

No Drawing.

Application filed March 4, 1927. Serial No. 172,927.

The invention relates to composition paper or pulp boards and methods of making the same, and has for its principal object the provision of an improved board of this character capable of use for making boxes, barrels, crates, cartons and cylinders, as well as a building material, such as siding, sheathing, roofing, or wall lining, which is capable of production in large quantities, may be made in varying degrees of stiffness, thickness, flexibility and strength, and is capable of economical production.

Another object is the provision of an improved process and method of procedure by means of which a material of this character may be produced by the use of waste or inexpensive materials, and, therefore, economically.

Other objects will appear hereinafter. I have discovered that the comparatively straight and strong fibers from the stems or stalks of certain plants, particularly the bagasse of sugar cane, may be combined, interlaced and felted with the comparatively crooked and branched fibers and pithy substances from the leaves of fleshy leafed plants, particularly the bagasse of the leaves of the sisal or henequen plant, and a strong, durable and efficient paper, or pulp board produced, of varying stiffness, thickness, flexibility and strength, adapted for various purposes, and at comparatively small cost.

I have learned that the fibers, particularly the smaller fibers, of the leaves of the sisal or henequen plant, owing to the fleshy nature of said leaves, are provided with a multitude of branching tendrils, branching from all four sides thereof and that these branching tendrils, when said fibers are reduced to a pulp, as in paper making processes, largely retain these branching tendrils, so that when interlaced and felted with the comparatively straight fibers of the stalks or stems of certain plants, particularly the bagasse of sugar cane plants, the branched tendrils interlock and interlace with the other fibers, thereby firmly binding the straight fibers together into a composition paper or pulp board of comparatively great strength and durability.

I have also discovered that the leaf fibers thus produced with branching tendrils have great tenacity, binding effect and flexibility, so that by varying the proportions of the leaf fibers to the stalk fibers, a board of

varying stiffness, thickness, flexibility and strength, may be produced to meet various commercial requirements.

As indicated above the material produced is, in substance and effect, a heavy, stiff, coarse and strong paper and, in general, is produced by subjecting such materials to an adaptation of ordinary paper making processes, especially combined as hereinafter set forth, to produce the desired results.

The process of preparation of the fibrous product or paper making material from the fibers and pith of comparatively straight and strong stalks, such as sugar cane or the bagasse of sugar cane is the process as specified in U. S. Patent 680,079, granted to George R. Sherwood Aug. 6th, 1901, or U. S. Patent 853,943, granted to Viggo Drewson May 14, 1907.

In certain other inventions utilizing bagasse and analogous fibers, and cooking the piths and fibers together, the cooking is usually arrested or discontinued at a temperature of 212 degrees Fahrenheit, or under, but I have found that at this low temperature, the lignum, gum and wax compounds are not destroyed, and I prefer to use the higher temperatures under pressure and also use a stronger caustic solution than is usually employed in such processes, such as are disclosed in the said heretofore mentioned patents. The treatment of the materials at the higher temperatures and with a stronger caustic solution will destroy the lignum, gum and wax compounds and thus, besides, freeing the fibers from the pith, destroys the food value of the composition to ants, insects, mice, rats, or the like, and thereby protects the resulting material from attacks by these vermin. Due to the better separation of the bundles of fibers and pith of the plants a product is ultimately obtained of smooth and uniform texture. The products thus prepared are conveyed to a storage and washing tank preparatory to being fed to a mixing tank, as hereinafter described.

As indicated, one of the purposes of my invention is to destroy, as far as possible, without too much weakening of the product, the lignum and gummy contents of the various fibers or piths, and thereby destroy the attraction for the food value of the completed product for ants, roaches, rats, mice and other vermin. To accomplish this pur-

pose the fibers, pithy substances, juices of the leaves and stalks of the fleshy leaved plants after being reduced to proper size are first cooked in a 60 percent caustic soda solution containing from 4 to 12 percent of the dry weight of the plant materials, from 1 to 3 hours and at a temperature in excess of 212 degrees Fahrenheit. As it is intended to use part of the natural resinous and gummy substance as a part of the binding and sizing required to unite the fibers and piths in the completed product, and as it is desired to use not less than 15 percent of the original resin or gummy matters, samples may be drawn off from time to time to test the cooking process and maintain proper control thereof. After this first cooking is concluded the material is conveyed by suitable means, to a storage and washing tank, preparatory to being fed to a secondary cooker in combination with the waste paper stock.

The waste paper stock having been originally cooked will not require any cooking or treatment except such as to render it sanitary and this can be accomplished by the second cooking when and as applied to and in combination with the fibers and pithy substances of the fleshy leaved plants as hereinbefore described. The waste paper stock having been reduced to required size by beaters, grinders or shredders, such as are generally used for this purpose is conveyed to a storage and washing tank preparatory to being fed to and cooked in the secondary cooker in combination with the fibers and pithy substance of the fleshy leaved plants as hereinbefore mentioned.

The waste paper stock, and the precooked fibers and pithy substance from the fleshy leaved plants having been washed, and freed from the excess of chemicals in cooking liquors, are fed from their respective storage tanks in the various amounts required to a secondary cooker, open to the atmosphere and equipped with agitators or mixing paddles, and the cooking liquors may or may not be composed of part of the spent liquors washed off in the previous cooking process, and sufficient water added. In this second cooking process the material is to be cooked for not less than one hour at a temperature of not less than 160 degrees Fahrenheit. The cooking in general does not differ materially from that generally used and well known in the manufacture of paper and pulp and the cooking may be performed by any of the generally used paper and pulp cookers purchasable in the open market.

After the stock has been sufficiently cooked in the second cooking process, it is drained to a mixing and cooling tank provided with paddles or agitators and there combined with the product or material as prepared under processes specified by Patents 680,079, or 853,943, mentioned above.

The combined products may be water-proofed or fireproofed by adding, while the stock is being mixed, any of the well known and generally used rosin or aluminum compounds commercially prepared for the purpose or purposes, or the product may be used without such water or fireproofing.

As to the proportions of materials used I prefer to use about 60 percent of the bagasse of sugar cane, about 20 percent of the bagasse of sisal leaves, and about 20 percent of waste paper stock. These proportions may be varied considerably depending upon the character of the product desired. The percentage of waste paper stock may be conveniently varied from 20 to 35 percent by bulk, the more paper stock being employed the smoother the resultant product will be. Likewise, the proportions of the stalk and leaf fibers may also be varied, the more stalk or stem fibers employed, the stiffer and stronger and more rigid will be the product. Conversely the more of the leaf fibers employed the more flexible and less brittle will be the product.

I also believe that the sources of the fibers may be varied within certain limits, using the stems or stalks of plants for the straight and strong fibers and the leaves of fleshy plants for the branching and binding fibers. Thus, it is thought, that corn stalks, or the stalks or trunks of the banana plant or palm tree may be employed for the straight fibers, and the leaves of such plants as the banana, palm tree, cactus and other plants having heavy and fleshy leaves may be employed for providing the branching and tenacious fibers.

The mixture of fibers and piths thus provided, and in the proportions as indicated, depending upon the results desired, are reduced to proper sizes by means of shredders, decorticators, grinders, beaters or pulverizing machines, such as are generally used for preparing fibrous materials for pulping in the paper making art, and are of standard manufacture and purchasable on the open market.

The mixture of fibers is then treated in ordinary paper or pulp making machinery to form the same into sheets or boards of sufficient and proper thickness for the purpose intended.

The processes of pumping, refining, beating, felting, pressing, compressing, cutting and drying of the paper or pulp board thus produced may all be efficiently and inexpensively accomplished by the use of any of the machines or apparatus marketed for the manufacture of paper, paper-board, pulp-board, or fiber board.

I prefer to use for felting purposes one of the many types of machine known as a wet machine having only one cylinder or as it is also known, a one cylinder mould, having only one foraminous surface, as this type of

machine will produce a more homogeneous material than machines having a multiple of foraminous forming surfaces.

The natural interlocking felting and weaving of the material during the felting processes as practiced for many years in the manufacture of paper pulp and fiber boards and the compacting or pressing under light pressure and the subsequent drying by any of the drying processes well known to the paper pulp or fiber board making art, the drying process evaporating the moisture from the pulpy wet material forms what are known as dead air cells and the resultant product can be used for insulating or sound deadening material.

In pressing the product to obtain varying degrees of hardness, the ordinary press rolls as generally used and known to the paper pulp or fiber board art may be used singly or in multiple to gain the desired effect.

While I have set forth and described the preferred composition of material and method of producing the same, these are capable of variation and modification without departing from the spirit of the invention. I, therefore, do not wish to be confined to the precise details set forth, but desire to avail myself of such variations and modifications as fall within the scope of the appended claims.

I claim:

1. A composition board of the class de-

scribed consisting of fibers obtained from the stems of sugar cane bagasse bound together by fibers obtained from the bagasse of sisal leaves, substantially as described.

2. The process of preparing a material of the class described consisting in separately cooking the fibers of the stems of plants and the fibers of the fleshy leaves of plants under pressure and at a temperature above 212 degrees Fahrenheit; mixing said leaf fibers with paper stock and cooking the mixture at a comparatively low temperature and atmospheric pressure; and then mixing all said fibers and forming said mixed stock into sheets by paper making processes, substantially as described.

3. The process of preparing a material of the class described consisting in separately cooking fibers of sugar cane bagasse and fibers of sisal leaves bagasse under pressure and at a temperature above 212 degrees Fahrenheit; mixing said sisal leaf fibers with paper stock and cooking the mixture at a comparatively low temperature and atmospheric pressure; and then mixing all said fibers and forming said stock mixture into sheets by paper making processes, substantially as described.

In witness that I claim the foregoing as my invention I affix my signature this 2nd day of March, 1927.

JOHN H. MITCHELL.